

## UNITED STATES PATENT OFFICE

1,959,734

PROCESS FOR PRODUCING PRACTICALLY  
PURE CELLULOSE (ALPHA-CELLULOSE)  
FROM RAW CELLULOSE OF ANY ORIGINFrancesco Carlo Palazzo and Fortunato Palazzo,  
Florence, ItalyNo Drawing. Application June 14, 1932, Serial  
No. 617,254. In Switzerland April 22, 1931

6 Claims. (Cl. 92—9)

Our present invention has for its object to provide certain new and improved processes for producing practically pure cellulose ("alpha cellulose") from raw celluloses of very different origin and composition, and remove from the latter the various substances usually accompanying alpha cellulose, by using reagents which, in the conditions chosen, do not alter in the least the alpha cellulose. The industrial use of our said invention, even on the largest scale, presents no difficulties at all nor requires special apparatuses.

Synthetically our said processes comprise a plurality of steps, each having certain features of its own, which succeed each other according to the following diagram:

- (1) Boiling in alkaline solution with sodium hydrate and sodium sulfite,
- (2) Bleaching of product from alkaline boiling with calcium hypochlorite or sodium hypochlorite in a neutral or slightly alkaline solution, or with potassium permanganate in a slightly acid solution, or with all of these systems together,
- (3) Removal of ashes from bleached product effected with sulfuric acid or hydrochloric acid,
- (4) Forming final product in preferred shapes according to purpose aimed at.

Only in case of having to obtain, for the final product, a particularly high degree of purity we insert between the second and third steps i. e. bleaching and ash removal, a fresh but less intense boiling with alkaline sodium sulfite solution for sodium hydrate.

As all of the operative steps, as said, have their own particular features, we are now going to describe same particularly, the more so as each of them is liable to modifications within well defined limits in relation to origin and composition of the raw cellulose under treatment, and qualities required for final product.

## 1. Cooking in alkaline solution

For this first step of process, besides its conditions proper, the following points are to be considered:

- (a) Condition of raw cellulose
- (b) Preferred heating system in digesters (with direct or indirect steam)
- (c) Concentration of liquor
- (d) Ratio between raw cellulose and liquor in as much as owing to the reciprocal influences in those conditions different operative modalities are to be chosen in different cases.

For the conditions proper of alkaline cooking, namely pressure and duration, the outer limits

are solely determined by the nature (origin and composition) of the raw cellulose under treatment, and according to such nature the working pressure may vary from 0,5 to 2,0 atmosphere, and duration from 1 to 3 hours.

For the other conditions there is, as said, a certain reciprocal interdependence which leads in each case to well defined operative modalities.

## (a) Condition of raw cellulose

The raw cellulose may be used both in air-dry condition in various shapes, and in wet condition with variable water tenor, that means that the raw pulp may be used partially dehydrated in centrifugal hydro-extractors (containing from 40%—45% of dry substance) or in suitable presses (containing from 30%—35% of dry substance) or a still more watery product (with only 20%—25% of dry substance) merely drained by dripping in tanks with perforated bottom.

In these different cases, except the diversities explained hereinafter relating to concentration of liquor and ratio between raw cellulose and liquor, the cooking may be started directly after admission of liquor to digester, whilst the procedure will be different in case of a raw cellulose such as immediately obtained from cooking of a ligneous material by the bi-sulfite or soda process.

In such case after the usual washings in the digester for removing the greater part of the waste liquor, the alkaline sulfitic liquor is admitted to digester on the already drained pulp, and circulated by a suitable pump from 5 to 6 times through the whole mass so as to mix same uniformly with the water imbibed by the raw pulp, and thus attain a uniform composition throughout said mass.

As to raw celluloses which are already in the shape of boards they are previously reduced to bands by a cutting device, or otherwise subdivided and then placed in the digester so as to obtain a comparatively compact charge on which the liquor is pumped at such concentration and in such quantity as will be indicated hereafter.

Digesters of various kinds may be used, such as horizontal, vertical or spherical, preferably rotating and permitting, when fixed, all the same an easy discharge of product and waste liquor. After cooking is completed the digester is discharged down in a tank with perforated bottom where the mass is left to drain for a short time by dripping, whereafter by repeated sprayings with water the greater part of the still impregnated waste liquor is expelled. The pulp thereafter passes to the pulper where it is further

washed and reduced to a pulp ready for bleaching.

In case of the raw cellulose to be treated directly obtained from the cooking of a ligneous material between the alkaline cooking and bleaching steps a series of mechanical treatments (screening, washing, refining) are inserted, wholly similar to those used for producing ordinary raw cellulose.

10

(b) *Heating of digester*

Heating of digester is preferably effected by indirect steam, but may also be effected by direct steam, and in the latter case the original concentration of liquor to be used for cooking is appropriately modified.

15

(c) *Concentration of liquor*

If the raw or starting material consists of raw pulp such as directly obtained from cooking of a ligneous material, merely washed in the digester, concentration of liquor is to be such as, also considering the ratio of raw cellulose to liquor to be finally a liquor of a tenor of 1% of NaOH and 0,5% of Na<sub>2</sub>SO<sub>3</sub>.

If f. i. between raw cellulose (supposed to be dry) and liquor there be a ratio of 1:10 and the raw pulp only contains 20% of dry substance, for each 100 kg. of dry substance (=500 kg. of wet pulp) 6 hl. of liquor are used, and the latter is to contain a total quantity of 10 kg. of NaOH and 5 kg. of Na<sub>2</sub>SO<sub>3</sub> so that after mixing the liquor (6 hl.) with the water imbibed by 100 kg. of dry substance (4 hl.) a liquor will be obtained which corresponds in volume to the above indicated ratio of 1:10, and contains 1% of NaOH and 0,5% of Na<sub>2</sub>SO<sub>3</sub>.

If, on the other hand, cooking instead of taking place with indirect steam is effected by direct steam injected into the mass, the quantity of condensation water to be produced in the digester when preparing the liquor must be taken into account, and therefore one must introduce into the digester a liquor of such concentration that together with the water already imbibed by the pulp, and with the condensation water of the direct steam, a liquor is obtained which contains, as above, 1% of NaOH and 0,5% of Na<sub>2</sub>SO<sub>3</sub>.

If the raw material instead of being raw cellulose in the form of sheets or boards the liquor to be used for cooking will have, in case of indirect steam heating, a concentration of 1,5% of NaOH and 0,5% of Na<sub>2</sub>SO<sub>3</sub>, and in case of direct steam heating a correspondingly higher concentration so as to obtain for the subsequent mixing with the condensation water of direct steam a liquor containing 1,5% of NaOH and 0,75% of Na<sub>2</sub>SO<sub>3</sub>.

20

(d) *Ratio between raw cellulose (supposed to be dry) and liquor*

This ratio is liable of some variation according to the condition of the material to be treated.

In case of highly watery material with a tenor water content of 75%-85%, the said ratio, as in the preceding example, will be 1:10, whilst in case of material which owing to having been squeezed out or centrifugated might have a somewhat lower water content, from 65% to 55%, a ratio of 1:8 may advantageously be kept, while leaving the concentration of NaOH (1%) and that of Na<sub>2</sub>SO<sub>3</sub> (0,5%) unvaried.

At least, in the particular case of air-dry product with 10%-12% of humidity being used, the most convenient ratio to be kept is 1:4, that is to say using 400 litres of liquor for 100 kg. of raw

product, which in spite of the higher concentration of the liquor (as prescribed at c, paragraph 4) implies an economy of reactives as for 100 kg. of air-dry cellulose 6 kg. (instead of 10 kg.) of NaOH, and 3 kg. (instead of 5 kg.) of Na<sub>2</sub>SO<sub>3</sub> are used.

2. *Bleaching*

According to the quality of the product to be bleached, and according to the more or less high degree of bleaching to be aimed at, jointly in any case with a comparative rapidity of the bleaching process, and with a low copper figure (always below 1,0) of finished product, bleaching of product from the alkaline cooking is effected with:

(a) Hypochlorite (of calcium or sodium) in a slightly alkaline solution, 85

(b) Potassium permanganate in a slightly acid solution, and

(c) A mixed hypochlorite and permanganate system, 95

(a) The hypochlorite solution containing from 1% to 2% of active chlorine besides a small quantity of calcium hydrate or sodium carbonate, which gives it a slight alkaline reaction, is caused to act at ordinary temperature on the pulp circulating in the pulper at a concentration not above 5%-6%. The bleaching is fairly rapid, and consummation of chlorine referred to 100 kg. of starting raw product does not, usually, exceed kg. 1. 100

(b) The chameleon solution of 1% of permanganate and 2% of sulphuric acid is also caused to act at ordinary temperature on the pulp circulating in the pulper at a concentration not above 5%-6%. The reaction is very rapid, and the consummation of permanganate,—which may be previously estimated by means of an analytical text,—does not usually exceed kg. 1.0 for 100 kg. of starting raw material supposed to be dry. 105

(c) The pulp at the above indicated concentration of 5%-6% is, before all, treated with the hypochlorite solution (at 1%-2% of active chlorine), only one half of the quantity of chlorine being used which would be necessary for complete bleaching. When the said quantity of chlorine is entirely absorbed (which only requires a few hours, even at ordinary temperature) to the said pulp, always circulating in the pulper, will be added a diluted solution (of 1%) of potassium permanganate slightly acidulated with sulphuric acid (2%) and in such quantity as to obtain a feeble reactive excess on the theoretical quantity of permanganate resulting from preliminary analytical test on the said pulp. After 15-30 minutes of circulation in the pulper the reaction will be completed, and there only remains carrying away the slight reactive excess, as also the manganese di-oxyd deposited on the fibres owing to the feeble quantity of sulphuric acid present. 110

3. *Removal of ashes from the bleached product* 115

In whichever way bleaching may be effected the removal of ashes from bleached product is equally effected with a diluted solution (0,5%-1%) of sulphurous acid acting both on the permanganate and respectively the manganese di-oxyd, 120 and on the small quantity of calcium carbonate or sodium carbonate deposited or, respectively, adsorbed in the fibre.

The treatment with sulphurous acid affected in the pulper and not prolonged beyond half an hour is followed by exhaustive washing of pulp, whereafter the product is ultimately subjected to various physical-mechanical treatments according to the shape to be given to final product. 125

## 4. SHAPING

(a) *Flakes and cotton wool*

After centrifugation of pulp in hydro-extractors followed by washing with distilled (condensation) water, the mass is comminuted and reduced to flakes which are ultimately brought to dry condition by carrying them on a suitable apron in counter-current to a hot air current. From the flakes thus obtained a cotton wool is prepared by subjecting them to a special mechanical treatment which, according to the fibres being to be kept long or short, will be effected either in a carding machine or in a centrifugal disintegrator.

(b) *Thin leaves or foils*

This shape is given the pulp in an ordinary continuous machine after previously refining it in the pulper if a product weighing less than 35 gr. for each square meter is to be obtained. The sheet or foil may then be wound on reel or variously cut, f. i. into narrow and short strips, or in narrow and long ribbons, and so forth.

(c) *Felt*

For preparing the cellulose in the shape of felt the fibre pulp is first treated in a rotary suction filter in which the rotation is controlled according to the thickness to be given to the felt, and the product fed on an endless apron is dried in counter-movement with an hot air current.

## Alkaline cooking of bleached product

As said, this cooking is only effected in case of a very high degree of purity being desired for the final product, such as to satisfy the most rigorous technical and analytical requirements. In such case however the cooking will be less intense, being effected at a pressure of 0.5-1.0 atm. and limited to a period of 1 hour.

As to the volume of liquor to be used, and its concentration, the same may be said as for the case of wet raw cellulose. As the bleached product after centrifugating or squeezing still contains from 55% to 65% of water, the liquor is to be of such volume and concentration that after being put together with the bleached product, between cellulose (supposed to be air-dried) and liquor there will be a ratio of 1:8, and finally a liquor will be formed containing 1.5% of NaOH and 0.75% of Na<sub>2</sub>SO<sub>3</sub> (or slightly more concentrated if heating be effected with direct steam).

Of course, if this treatment is to be applied to the product already bleached, the preceding bleaching may be effected by using a slight excess of oxydant. In this way, in the case of wood cellulose, the last traces of lignine will be completely removed, whilst the small quantity of oxydellulose which may be formed owing to said excess, does not ultimately go to contaminate the bleached product because it goes into solution in the subsequent alkaline-sulfite treatment.

A particular feature of the above described boiling consists in the recovery of the greater part (75%-80% in volume) of the waste liquor, the said recovery being effected, for one portion, by leaving the mass to drip into a tank with perforated bottom, and for the remaining portion by subjecting the drained product to centrifugating or squeezing. In this way a total quantity of liquor is obtained sufficient for effecting therewith the first cooking of a quantity of raw cellulose equal to that from which the bleached

product was obtained, and such cooking process quite normally as the liquor besides the two unaltered reactives NaOH and Na<sub>2</sub>SO<sub>3</sub> duly contains a very small quantity of organic substance.

As to the centrifugated or squeezed product, this is treated for a short period in the pulper and finally for the removal of the ashes therefrom, or in the above said way with sulphurous acid or, in an analogous way with an equivalent quantity of hydrochloric acid.

Having now particularly described and ascertained the nature of our said invention and in what manner the same is to be performed, we declare that what we claim is:

1. Process for producing, from raw cellulose of any origin, practically pure cellulose with 96% up to 99% of alpha-cellulose, copper figure from 0.8 to 0.2, ether-soluble substances from 0.15 to 0.05% and ashes from 0.18% to 0.10%, which process consists in cooking said celluloses in the most variated conditions, wet or air-dry, purified or not purified, in a digester with an alkaline-sulfitic liquor containing from 0.5 to 1.5% of NaOH and from 0.25% to 0.75% of Na<sub>2</sub>SO<sub>3</sub>, under a pressure from 0.5 to 2 atm., and for a period variable between 1 and 3 hours; the material obtained from the said cooking at a concentration of 5% to 6% being thereupon bleached at ordinary temperature with a diluted potassium permanganate solution of 1%, acidulated with 2% of sulphuric acid.

2. Process for producing, from raw cellulose of any origin, practically pure cellulose with 96% up to 99% of alpha-cellulose, copper figure from 0.8 to 0.2, ether-soluble substances from 0.15 to 0.05% and ashes from 0.18% to 0.10%, which process consists in cooking said celluloses in the most variated conditions, wet or air-dry, purified or not purified, in a digester with an alkaline-sulfitic liquor containing from 0.5 to 1.5% of NaOH and from 0.25% to 0.75% of Na<sub>2</sub>SO<sub>3</sub>, under a pressure from 0.5 to 2 atm., and for a period variable between 1 and 3 hours, the product thus obtained being then treated in a digester with an alkaline-sulfitic liquor at a pressure of 0.5 to 1.0 atm. and for a period of 1 hour; the material obtained from the second cooking with alkaline-sulfitic liquor being furthermore treated at ordinary temperature with a diluted solution of sulphurous acid 0.5% to 1% or other equivalent hydrochloric acid solution, and ultimately subjected to exhaustive washing in the pulper.

3. Process as claimed in claim 2, characterized in that the final product obtained from said chemical treatments is furthermore subjected to suitable physical-mechanical treatments so as to form the same at will in the shape of flakes, cottonwool, thin sheets or leaves, reels, bands, ribbons or felt.

4. Process for producing, from raw cellulose of any origin, practically pure cellulose with 96% up to 99% of alpha-cellulose, copper figure from 0.8 to 0.2, ether-soluble substances from 0.15 to 0.05% and ashes from 0.18% to 0.10%, which process consists in cooking said celluloses in the most variated conditions, wet or air-dry, purified or not purified, in a digester with an alkaline-sulfitic liquor containing from 0.5 to 1.5% of NaOH and from 0.25% to 0.75% of Na<sub>2</sub>SO<sub>3</sub>, under a pressure from 0.5 to 2 atm., and for a period variable between 1 and 3 hours; the material obtained from cooking in a concentration of 5 to 6% thereupon being bleached at ordinary temperature with a diluted solution of calcium or sodium hypochlorite, containing 1 to 2% of effective chlo-

rine besides a small quantity of calcium hydrate or, respectively, sodium carbonate and, after washing, again treated at ordinary temperature with a diluted solution at 0.5 to 1% of sulphurous acid, whereupon an exhaustive washing in the pulper is effected.

5. Process for producing, from raw cellulose of any origin, practically pure cellulose with 96% up to 99% of alpha-cellulose, copper figure from 10 0.8 to 0.2, ether-soluble substances from 0.15 to 0.05% and ashes from 0.18% to 0.10%, which process consists in cooking said celluloses in the most variated conditions, wet or air-dry, purified or not purified, in a digester with an alkaline-sulfitic liquor containing from 0.5 to 1.5% of NaOH and from 0.25% to 0.75% of Na<sub>2</sub>SO<sub>3</sub>, under a pressure from 0.5 to 2 atm., and for a period variable between 1 and 3 hours; the material obtained from cooking in a concentration of 5 to 20 6% thereupon being partially bleached at ordinary temperature with a diluted solution of hypochlorite of calcium or sodium containing from 1 to 2% of effective chlorine besides a small quantity of calcium hydrate or, respectively, sodium carbonate, and then, after washing, finally bleaching at ordinary temperature with a diluted so-

lution, at 1%, of potassium permanganate, acidulated with sulfuric acid of 2% strength.

6. Process for producing, from raw cellulose of any origin, practically pure cellulose with 96% up to 99% of alpha-cellulose, copper figure from 80 0.8 to 0.2, ether-soluble substances from 0.15 to 0.05% and ashes from 0.18% to 0.10%, which process consists in cooking said celluloses in the most variated conditions, wet or air-dry, purified or not purified, in a digester with an alkaline-sulfitic liquor containing from 0.5 to 1.5% of NaOH and from 0.25% to 0.75% of Na<sub>2</sub>SO<sub>3</sub>, under a pressure from 0.5 to 2 atm., and for a period variable between 1 and 3 hours; the material obtained from cooking in a concentration 85 90 of 5 to 6% being first bleached and then, after washing, treated in autoclave with an alkali-sulfitic liquor at a pressure of 0.5 to 1.0 atmosphere for a period of 1 hour; washed again, and finally treated with a diluted solution at 0.5 to 1% of sulphurous acid or another equivalent solution of hydrochloric acid, and exhaustive washing in pulper.

FRANCESCO CARLO PALAZZO. 100  
FORTUNATO PALAZZO.

|    |     |
|----|-----|
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |